

R. S. Stanton

Making Steel

No 88,524.

Patented Mar. 30, 1869.



Witnesses;  
A. Geiger  
R. Cooper

Inventor;  
R. S. Stanton



ROBERT S. STENTON, OF BROOKLYN, NEW YORK.

*Letters Patent No. 88,524, dated March 30, 1869; antedated March 25, 1869.*

IMPROVEMENT IN THE MANUFACTURE OF STEEL DIRECT FROM THE ORE.

The Schedule referred to in these Letters Patent and making part of the same.

*To all whom it may concern:*

Be it known that I, ROBERT S. STENTON, of the city of Brooklyn, county of Kings, State of New York, have invented an Improved Method of Manufacturing Steel-Sponge, and Steel direct therefrom.

The usual processes by which cast-steel is made are all more or less circuitous.

By one, the most reliable, the ore is first roasted, then smelted in a blast-furnace, to make it into pig-iron, where it is carbonized, then refined. The refined metal is made into malleable iron, in a reverberatory furnace, where it is decarbonized. The bars so made are then again carbonized, either in a converting-furnace, or in the crucible, in which they are melted, and from which is poured the cast-steel ingot.

Cast-steel, the product of malleable iron, made in a sinking-fire, avoids the smelting process.

Cast-steel, made by the Bessemer and Martin processes, avoids the intermediate stage of malleable iron; it is made direct from the pig.

I propose, by my invention, so to treat large masses of suitable iron-ore, that when placed in a properly-constructed furnace, and subjected to a due degree of heat, it will melt, and the product thereof be cast-steel, of various degrees of hardness, down to softest decarbonized cast-steel, at the will of the manufacturer.

The nature of my invention consists in charging a kiln, or oven, or in packing a heap, or hill with ore, fuel, and carbon, as hereafter described, in order to accomplish certain essential results in a new and superior manner, viz, to deoxidize, to cleanse, and to carbonize metallic ores, more particularly black oxides, and other suitable descriptions of iron-ore, producing, as a result, a metallic sponge, that, where iron-ore has been used, will have become a sponge of steel, fig. 3, owing to the carbonizing-process that has been carried on with the deoxidizing and the cleansing-process.

Ore prepared in this manner is no longer iron-ore, but becomes really metallic steel, and requires only to be melted in a properly-constructed furnace, to be run into ingots of any size, for any purpose, from a needle to a railway-bar, or from a railway-bar to a canon of the largest dimensions, and that at a cost but little, if anything in advance of the present cost of good charcoal pig-iron.

Iron-ore has been deoxidized, and a sponge of iron has been made in various ways—by mixing iron-ore and fuel in heaps, on the ground or in kilns, and firing the same, or by passing the waste gases from a blast-furnace head, through masses of iron-ore placed in a proper receptacle.

Sponge, of steel, has been made by the cementation of ore in an air-tight oven, or pot, in the same way that blistered steel is made from malleable iron.

My invention is an improvement on both of these old processes.

By my new method, I produce sponge of steel in

an open kiln, or oven, or even in a heap, or mound. This latter, however, being less under control, the results will not be uniform, and it will not be advisable to have recourse to it.

To enable others skilled in the art to make and use my invention, I will proceed to describe the same.

Figure 1 is a sectional elevation, showing a small portion of fuel, carbon-ore, carbon-fuel, &c., in alternate layers.

Figure 2 is the same, with the fuel between every two layers of ore and carbon.

Figure 3 is a view of a sample of steel-sponge, partially polished on one side, to show its metallic structure and nature.

Like letters of reference indicate corresponding parts. The object of my invention is to make sponge, of steel, in large masses, at the least possible expense.

This can be done in almost any kiln in which charcoal can be made.

I do not, therefore, at this time, claim any particular construction of furnace, kiln, or oven, but a method of packing, or charging, or of manipulating ore in any such furnace, kiln, or oven in which the requisite heat can be obtained.

First, this consists in placing layers, or alternate layers of fuel, wood or peat, in preference to coal, as shown at A in figs. 1 and 2; carbon, (fine charcoal,) as at B, figs. 1 and 2; ore, by preference broken small and separated, as at C, figs. 1 and 2; carbon, as at D, figs. 1 and 2; and then again fuel, A, as in figs. 1 and 2; or, at the option of the operator, the fuel, A, may be placed, as in fig. 2, between every second layer of carbon and ore, or even between every third or other number of layers, the object being to obtain a bright but not a melting-heat, gradually rising up through the mass. Enough, and no more, of wood, or other fuel, must be used than is needed to accomplish this purpose.

The topmost layer should be one of fuel, and the whole must be enclosed, or covered in with masonry, or earth, or sand, the supply of air being regulated in such a way that combustion shall be even and regular.

At intervals of twelve inches, or thereabout, and all round the sides, the beds of ore should have spaces, E, of about one inch in diameter, (see figs. 1 and 2,) into which a handful of small charcoal must be inserted, for as cementation goes on, the ore will slightly fuse, and weld into a cake.

The oven, or kiln should be so arranged that the gases of combustion and carbonization will pass away downward, which, without these vents, it would be almost impossible for them to do. This, however, though preferable, is not an essential.

I use either a natural draught, or apply a blast to stimulate combustion, dependent on the construction of the kiln, or furnace. The gases generated by a suitable arrangement of flues and manipulation of the

furnace, can be saved, and utilized as heat-producers, when combined with a further supply of air, heated or cold, or air and steam, as found expedient.

The layers of fuel should be in sufficient quantity to heat the ore to a white, but not to a melting-heat; the ore placed in layers two inches thick, the carbon half an inch to one inch above, and before each layer of ore, or be mixed equally through it, in proportions dependent on the description and chemical components thereof.

One hundred tons of steel-sponge or more can be made at one time.

Second, having explained the method of making steel-sponge, by the process of deoxidizing and carbonizing iron-ore, by a peculiar arrangement of the component materials used, I will now proceed to describe another method of accomplishing the same object by a different and more rapid, but equivalent process.

As already stated, ores of iron have been deoxidized and made into a sponge of iron, by being packed into a proper receptacle, and forcing the waste heat or gases from the blast-furnace head to pass through the same, until the oxygen, and as much of the other impurities of the ore had been expelled, as could be driven off without subjecting it to a fusing-heat.

Iron-ore, at a white heat, will rapidly absorb carbon when it is placed in juxtaposition with it. When, therefore, the body of ore is at this point, (I do not, of course, confine myself to using heat obtained by economizing the waste of the blast-furnace,) I throw into the heated mass a stream or streams of carbonaceous gas obtained from proper auxiliary apparatus.

Wherever the carbon can attack the heated ore, it will do so, and a sponge of steel will be the result.

Furnaces can be so arranged as to be fed with ore at the mouth, discharging the sponge at the foot, the ore being heated, deoxidized, and carbonized in the one part, but cooling sufficiently below to allow of being raked out at proper intervals; or fuel, and then ore and carbon may be alternately charged at the

mouth, and after the ore is sufficiently deoxidized and carbonized, it can be discharged at the foot, and thus the operation be made continuous.

My claim being for a novel method of treating metallic ore in furnaces, kilns, &c., that are not air-tight, being neither ovens, muffles, nor retorts, to make steel-sponge, and not being for any form of furnace, or for anything, but simply for the process of making such sponge in the manner set forth, and to smelt or melt the same, the construction of the furnaces, or kilns, and the method, or methods by which the carbonaceous gases required for the second of the methods described are generated, and the apparatus and material used, are properly the subjects of separate patents, and therefore not here set forth.

In melting the sponge, made as herein described, I mix with the same such a proportion of pig-iron as may be requisite to supply an increased percentage of carbon, when such is required, using also as a flux and detergent, the oxide of manganese.

The carbon, or fine charcoal, instead of being put above and below the ore, may be mixed with it, and then placed in juxtaposition with the fuel, as hereinbefore stated.

By care in the degree of carbonization, and a proper management of the furnace, a natural, a puddled, a semi-steel, or even a malleable-iron loop may be produced from this sponge, either alone, or in combination with pig-iron, in a reverberatory furnace.

What I claim as my invention, and desire to secure by Letters Patent, is—

The process, or method, herein described and illustrated, of making steel, by heating the iron-ore with fuel and charcoal, arranged in alternate layers, thus producing steel-sponge, and by reducing said sponge, substantially in the manner hereinbefore set forth.

R. S. STENTON.

Witnesses:

A. JAEGER,  
H. JAEGER.